

# UNITED STATES PATENT OFFICE.

VICTOR G. BLOEDE, OF CATONSVILLE, MARYLAND.

## COMPOUND TO BE USED AS AN ADHESIVE IN THE MANUFACTURE OF ENVELOPS AND THE GUMMING OF PAPER.

1,198,099.

Specification of Letters Patent. Patented Sept. 12, 1916.

No Drawing.

Application filed February 28, 1914. Serial No. 821,786.

*To all whom it may concern:*

Be it known that I, VICTOR G. BLOEDE, a citizen of the United States, residing in Catonsville, in the county of Baltimore and State of Maryland, have invented a new and useful Compound to be Used as an Adhesive in the Manufacture of Envelops and the Gumming of Paper, of which the following is a specification.

10 In the manufacture of envelops and the gumming of paper artificial, or natural gums soluble in water are used, the former usually being produced by the hydrolyzation of some form of starch, and called 15 dextrin or gum, the latter natural products as represented by gum arabic, senegal, etc. These products are all used in the form of a thick syrupy solution of various degrees of density and produced by dissolving the 20 dry gums by boiling with water, a process well known by all manufacturers using such products.

While the ordinary grades of paper present no difficulty in the matter of perfect adhesion, there are a considerable number of 25 grades which owing to some peculiar texture or construction, or through the character of the stock or sizing employed in their manufacture, high compression, or finish, or other 30 causes show a remarkable degree of resistance, or repulsion for the gum used to effect their adhesion, and in many instances are so refractory that the paper cannot be made to permanently adhere. Envelops 35 made from paper of this type open up with the greatest ease, and in some cases, and especially after a few weeks' storage, the gummed surfaces separate or fall apart, making the envelop useless commercially. 40 Among the types of paper especially subject to this trouble may be named the hard sized linen and Manila grades, also certain embossed or highly calendered or finished papers.

45 Papers of the type described, while often in other respects especially adapted for envelops or other manufactured products, present almost insurmountable difficulties when it comes to properly sticking one surface upon the other. It has long been known that caustic soda or potash, or other strong alkali added to the gum used in working these papers will produce satisfactory results so far as adhesion is con-

cerned, but the use of such agents is in 55 most cases entirely inadmissible owing to the discoloration they produce in the gum itself as well as white or colored papers. Working upon the theory that the faulty adhesion was due to the water-proofing of 60 such paper either through great compression of the fiber, natural oils, or waxes, or fatty or resinous matters used in sizing, numerous trials were made to overcome this difficulty by the addition of some substance 65 having strong power of penetration as well as affinity for, or solvent action upon, substances, or conditions, producing the water repellent effects in these refractory papers. It was found as a result of these trials that 70 any substance having a solvent action on fatty resinous, or waxy bodies when added to and combined with the gum used as an adhesive increased its sticking qualities to such an extent as to make satisfactory results possible with grades of paper hitherto 75 regarded as "unstickable." Another great practical advantage incidentally brought about by such an addition is the fact that owing to the water repellent condition of 80 the paper being overcome by its action, or penetrating properties, the gum applied forms a much smoother and more slightly film, and the puckering or buckling of the paper is greatly lessened, producing very 85 much better and more satisfactory work.

Among the substances that are applicable in my process, I may name any of the volatile hydrocarbons, such as benzin, benzol, turpentine, chloroform, ether, tetra chlorid or bisulfid of carbon, indeed, as stated, any volatile solvent of fatty or resinous matters. I do not, therefore, confine my claims to any special substance or compound, but have found in practice that tetra 90 chlorid of carbon, owing to its uninflammability, ready volatility without leaving any odor whatever, and low cost answers my purpose rather better than most other substances of the type named. Some non- 100 volatile oils and their saponifications, or emulsions, also produce similar effects, for instance, the sulfo-ricinates, but not nearly in so marked a degree, and possess the further objection of remaining in the composition while the volatile additions named 105 wholly disappear by the time the applied watery solution of gum has dried.

In carrying out my process, I first make up a solution of a gum or dextrin of the desired concentration or viscosity. The relative amount of water and dry material used depends somewhat upon the character of the product from which the solution is made, as there is a wide range in the viscosity of the various starch gums on the market, but I have found that from one and a half pounds to two pounds of the dry gums or dextrin of commerce to one pound of water will give good results. In actual practice, I use what is termed the standard envelop gum, and make up my mixture as follows: 160 lbs. standard envelop gum, 100 lbs. water.

Sift the gum into the water cold, and stir the mixture until a smooth paste is formed, free from lumps and clots of undissolved material. Heat this mixture in a copper jacketed kettle, preferably provided with a mechanical stirrer, and after having brought it to a boil, simmer the mixture for one to one and one-half hours, then allow to cool to normal temperature, and having replaced the evaporated water so as to bring the mixture back to weight of both ingredients, that is, 260 lbs., add 5% to 10% of the dry weight of the gum used, that is, 8 lbs. to 16 lbs. of tetrachlorid of carbon, benzol, turpentine, or similar solvent, and stir the composition until a full combination, or emulsification of the solvent with the paste has

been effected, when the composition is ready for use, and may then be applied in the ordinary manner known to the trade.

I do not limit myself to any specific solvent, nor to specific proportions in which it is to be used, as both the choice of the agent employed and its quantity used depends largely upon the character of the paper operated upon, but as stated, I have found tetrachlorid of carbon a very satisfactory agent and an addition of 5% of the weight of the liquid gum a satisfactory proportion for general work.

While I have especially mentioned artificial and natural gum solutions, these being most largely used for this purpose, my process is equally applicable to preparations of glue or flour or raw starch pastes used as adhesives in some classes of work, the addition of the solvent besides securing the advantages set forth, also acting as a powerful preservative and preventing fermentation and decay.

I claim:

A water soluble mucilage or paste consisting of about 160 pounds of envelop gum, 100 pounds of water, and eight to sixteen pounds of volatile solvent, substantially as described and for the purpose specified.

VICTOR G. BLOEDE.

Witnesses:

Wm. H. THOMAS, Jr.,  
H. M. YOE.

Copies of this patent may be obtained for five cents each, by addressing the "Commissioner of Patents, Washington, D. C."